

## UNITED STATES PATENT OFFICE

2,314,658

## PROCESS OF PREPARING WOOD PULP

Fredrich Olsen, East Alton, Ill., assignor to The  
Cellulose Research Corporation, East Alton, Ill.,  
a corporation of Delaware

No Drawing. Application January 20, 1939,  
Serial No. 252,042

2 Claims. (Cl. 92—16)

This invention relates to the preparation of high grade cellulosic material from wood.

The object of this invention is to provide a process for the production of wood pulp having a high alpha cellulose content.

Another object of this invention is to provide a process for the production of wood pulp of high quality, suitable for use in preparing cellulose derivatives; for example, cellulose nitrate or xanthate.

Another object of this invention is the production of high quality wood pulp for use in the manufacture of paper having good stability.

The process comprises gradually reducing the soda soluble and pentosan content of the wood pulp and concomitantly attaining a high alpha cellulose content, usually above 98%. The wood cellulose produced is a homogeneous product which renders it well adapted for derivative purposes and for the preparation of high stability paper pulp.

The process of this invention subjects the wood to a series of treatments specially designed to attain a condition of maximum purity without the formation of undesirable degradation products. This is in direct contrast with prior and present day practice wherein the entire burden of purifying the cellulose from the very complex, woody structure rests on only a few processing steps, necessarily drastic in character, in order to obtain high purity; or where mild in character, resulting in a sacrifice of purity of product. The conventional manufacturing technique in the preparation of wood pulp is based upon the use of a very small number of pieces of standard equipment; viz., digesters, washers and bleachers. The engineering plan back of such equipment is evidently the production of as large yields as possible of white fiber. Even the cotton linters purified for use in derivatives employ substantially the practices of the manufacturers of bleached soda pulp as used in book paper. In contrast, the process of the current invention aims at a specially coordinated set of systematic and specific chemical treatments to remove the individual impurities associated with the cellulose in the raw, woody material.

This series of treatments comprises impregnating wood with an aqueous solution, such as an acid or alkaline delignifying reagent, at a temperature lower than that at which lignin is removed from the wood, digesting the impregnated wood at suitably elevated temperature until a sufficient amount of the inter-fiber binding material has been removed to permit separation of the wood into individual fibers, bleaching the wood pulp so obtained by treatments including chlorination, alkali and hypochlorite, treating the bleached pulp with caustic soda solution at

elevated temperature and thereafter subjecting the bleached pulp to a mercerizing treatment.

When especially high whiteness and low pentosan content of pulp is desired, the mercerized pulp after water washing is thereafter again mercerized.

For the purpose of removing certain impurities comprising non-fibrous material, such as coagulated protoplasm, cell wall debris, small particles of resin and the like, it has been found desirable to subject the pulp to a classifying treatment in which such "fine" material is separated and removed from the long fiber portion. This permits an attainment of a better color in the final product and its derivatives or a greater stability in the resulting paper.

In the process of this invention, an intimate association of digesting liquors having proper reactive strength, and at the same time nearly uniform distribution of the delignifying chemicals throughout all portions of the wood, is attained before providing reactive temperatures, so that when the proper temperature is reached, the reaction proceeds rapidly and simultaneously throughout all portions of the wood, including the difficultly penetrable centers of the wood subdivision.

Before such uniform impregnation can be attained, it has been found necessary to remove the air from the interstices of the wood. This is accomplished by first boiling the wood suitably subdivided in a liquid wherein the vapor of the liquid replaces the air within the interstices of the wood. The liquid may be the delignifying reagent itself, such as a caustic soda solution, kraft liquor and the like, or it may be water; or it may be an electrolyte solution having a concentration of electrolyte tending to inhibit any reaction or adsorption of the delignifying reagent at boiling temperature.

After the removal of air from the subdivisions, they are maintained submerged in the delignifying reagent of suitable concentration to give the desired bleachability in the cooking schedule employed until they are uniformly impregnated with said delignifying reagent either by condensation of the vapor within the voids and/or by diffusion. After the wood has been uniformly impregnated with the delignifying solution, the temperature of the wood subdivisions is then raised and the digestion continued until the desired bleachability of raw material is attained.

The viscosity of cellulose solutions has long been considered as associated with a state of complexity of the cellulose molecule. The change in viscosity of the cellulose molecule seems to require two conceptions:

1. The change in viscosity obtained by separating the long chain molecules in the bundles from each other by destroying the secondary

valence forces. This action will be referred to as "splitting."

2. The reduction in viscosity obtained by depolymerization, which involves breaking the primary valence bonds and reducing thereby the chain lengths of the cellulose molecules. This action is described as "scission."

The purification treatments of the wood pulp obtained as described above are preferably carried out under conditions which result in altering 10 the viscosity by splitting of the secondary valence forces rather than by scission of the primary valence bonds, since the latter appears to result, in most cases, in the formation of undesirable quantities of degradation compounds. Thus the 15 pulp is given a mild chlorination, preferably with an amount of chlorine reacting only with the lignin content and which will be substantially exhausted in a period of about 20-30 minutes. The products of the chlorination, such as chlorinated lignin or the like, are then removed from the pulp, for instance, employing a dilute alkaline solution and water washing.

The bleaching treatments given the pulp are preferably very mild in their nature; the conditions being controlled to avoid any degradation other than that necessitated by the reduction in viscosity desired.

The treatment of the bleached pulp with alkali at elevated temperature is carried out in such a manner as to remove the maximum amount of non-cellulosic impurities with minimum degradation of the cellulose. It has been found that concentrations of 5%-9% sodium hydroxide in solution are preferable.

When mercerizing the pulp, concentrations of caustic soda from 10%-18% and temperatures in the range of 20°-40° C. have been found satisfactory.

When wood is subjected to the successive treatments described above, the resulting cellulose product is in an ideal condition of purity, molecular complexity and permeability to reagents for conversion into high quality derivatives. The physical state of the fiber is such that reagents penetrate readily into the individual cell particles. Conversion reactions commence at the surface of these particles and proceed rapidly into their interior by diffusion of the reagent through the available inter-molecular spaces, thus leading to a highly uniform product.

As described above, I may use any of the known alkaline and acid delignifying reagents, but in any case the practice of properly relating the reagents and woody material prior to attaining reactive temperatures by the removal and exclusion of the normal air content of the wood is important where uniformity in impregnation is to be attained.

When the pulping of the wood and its purification have been conducted under especially lenient conditions, as described above, designed to effect a separation of the bundles of long chain molecules by splitting, i. e., destroying the secondary valence forces and largely avoiding the depolymerization of the cellulose through scission or the breaking of primary valence bonds, the effect of such uniform, mild treatment on the pulp is to attain an end product distinguished from all products of the prior art processes, among other things, by its homogeneity.

The following examples describe two specific embodiments of the invention, but it is to be understood that the invention is not limited to the specific details set forth therein.

I may use maple, aspen, tulip and other varieties of poplar, yellow birch and other suitable species of wood. In any case, care is used to select wood as free as possible from knots, decay and other impurities. The bark is carefully removed, and the wood thoroughly washed.

#### Example A

Yellow birch, for example, is reduced either to the flake or chip form of subdivision. The digester is filled with yellow birch chips of approximately half inch length, and the chips are boiled at atmospheric pressure in a solution of aluminum sulfate of about  $10^{-5}$  molar, after which the liquid is allowed to cool to a few degrees below the boiling point, for instance, 97°-98° C. The time of treatment is preferably about one hour to allow for the removal of air and the deposition of the electrolyte in the deaerated cavities of the wood, and after this is completed, the batch is allowed to stand for one hour, the chips during this period remaining submerged.

The solution is then drained from the wood and a caustic soda solution added until the ratio of liquor to wood is 3.25 pounds to 1 pound. The concentration of the caustic solution is so adjusted that after taking into consideration the amount of liquid present in the pretreated chips, the ratio of chemical to wood in the system will be approximately 0.2 pound of NaOH to 1 pound of wood. If the greater degree of homogeneity of product resulting from digestion which has been performed on chips preimpregnated with an electrolyte as described above is not required, this electrolyte treatment may be omitted. In this case, the chips are boiled in the alkaline digesting liquor of approximately 0.2 pound NaOH to 1 pound of wood (ratio of liquor to wood approximately 3.25 to 1) under freely vented conditions, or as described in copending application, Serial 17,894, filed April 24, 1935, now issued as U. S. 2,137,779, until uniform distribution of the delignifying agent throughout the wood has been secured.

45 The caustic soda solution is added to the digester at 70° C. or higher, and after the chips are submerged by this liquor, heating and circulation are started by means of a circulation pump which draws off the liquor at the bottom of the digester and charges it into the top through a circular perforated pipeline located at the top of the cylindrical section of the digester while high pressure steam is simultaneously introduced into the bottom of the digester at a temperature of approximately 200° C. The relief valve on the digester is "cracked" throughout the initial steaming to permit the air above the liquor level to escape and avoid any false pressure. The temperature rise of the mass is halted at about 96°-98° C. and maintained at this point for one hour. This pause permits the caustic to penetrate the chips without reaction and at a temperature below boiling, tending to preserve the electrolyte deposit, and at the same time sufficiently high to expedite the entry of the caustic into the interstices of the wood. The relief valve is then closed and the temperature raised to 160° C. as rapidly as the facilities will permit, the usual requirement being from 1½ to 2 hours. The temperature is held between the limits of 160° C.  $\pm$  2° for 6 hours. The liquor circulation pump is stopped 55 15-20 minutes before the termination of the cook so that incoming steam may break up any packing of the pulp that sometimes occurs and tends to prevent the blowing of the digester cleanly. At

the end of the cooking time, steam is shut off and the pressure in the digester, which is usually about 75 pounds per square inch, is utilized to discharge the pulp through the blow valve located in the bottom of the digester, the stream of pulp usually being directed at a steel target in the blowpit, which impact serves to largely break down the chips into a pulpy mass. As soon as the blow valve is opened, waste black liquor from a previous digestion is pumped into the digester for about 15 minutes to assist in attaining a clean blow or discharge of the pulp. The pulp may be washed in the digester with the exclusion of air and discharged into a dump-tank provided with mechanical means by which the pulp is subjected to violent agitation to break down any bundles of fibers which may exist. This type of digestion involving special impregnation with the digestion liquors and particularly when electrolyte preimpregnation has been practiced has effected the production of a raw pulp which is more homogeneous in composition and structure than that resulting from conventional digestion practices. The impurities which remain are more uniformly distributed throughout the pulp and more readily accessible to the subsequent purification reagents. Unless the digestion treatment has produced a raw pulp of this type, subsequent purification steps are inadequate in effecting proper removal of certain kinds of impurities.

The pulp is now ready for purification and is first treated at 3.5% consistency with the equivalent of an amount of standard bleaching powder in the form of chlorine water which will substantially exhaust in 20-30 minutes. The treatment is preferably carried out at 20°-22° C. In order to utilize the acids formed by the chlorination treatments, as a means of removing ash from the cellulose, the treatment is allowed to continue for a total of 45 minutes. A convenient and desirable concentration of chlorine water to use is 5 grams of chlorine per liter.

At the end of the 45 minute chlorination treatment time, a sufficient amount of sodium hydroxide is added to the slurry to give a 1% NaOH concentration and a treatment consistency of 2%. It is desirable to keep the concentration of the sodium hydroxide solution added to the pulp slurry at 7% or less in such an amount as to give a slurry in which the final concentration is about 1% NaOH. I have found that caustic solutions stronger than 7% have a tendency to "set" the chlorinated compounds and make them more difficult to remove. An unfavorable consequence of the "setting" of the chlorinated compounds is that a relatively drastic oxidation treatment is necessary to attain the desired high white pulp color, and this results in a reduction in the viscosity of the final product. The pulp is treated for 30 minutes at 100° C. The mass of pulp is then promptly transferred to a continuous filtering device or a centrifuge and washed thoroughly with purified water until the pH of the slurry is between 7.0-8.0 units.

The pH of the pulp slurry coming from the diluted alkaline boil is a very important factor and must be closely controlled. If the pH varies between 7.0-8.0 units, it should be adjusted by the addition of either hydrochloric acid on the one hand or caustic soda or lime on the other. Calcium hypochlorite, containing the necessary amount of available chlorine to reduce the permanganate number of the pulp to approximately 0.6 and to reduce the cuprammonium viscosity to a value in the range desired in the final product,

is then added to the pulp slurry; the consistency having been adjusted to 3.5% and the temperature to 21°-23° C. and then allowed to react for approximately 4 hours. The bleaching powder is added in the form of a solution containing 58-62 grams of bleaching powder per liter and saturated with calcium hydroxide. I have found that the degrading effect of the oxidant can be held at a minimum by bleaching at relatively low temperatures, for example, 20°-25° C. and at high pH, for instance 8.5-11.0 units. After the completion of the bleach, the pulp is washed free of available chlorine, as indicated by testing with starch iodide paper.

15 After this washing treatment, the pulp is immersed in a concentrated sodium hydroxide solution of 7.0%  $\pm$  1% at a consistency of 4% for a period of 3 hours at 100° C. This treatment should be carried out under conditions which 20 will allow the minimum amount of atmospheric oxygen to come in contact with the pulp. When the alkaline boil is completed, the solution is drawn off and the pulp washed with purified water until the pH has been reduced to between 7.0 25 and 8.0 units. This sodium hydroxide treatment effects important changes in the alpha and soda soluble contents of the pulp.

Pulp at this point is satisfactory for the manufacture of certain grades of paper, but where 30 superior qualities of paper and derivatives are desired, additional purification treatments are essential, and the treatment with calcium hypochlorite previously described is now repeated.

After the second bleaching treatment, the pulp 35 is thoroughly washed in purified water as after the first bleaching. It is then immersed and thoroughly agitated in a 13.7% NaOH solution at 25° C. for 1 hour at 4% consistency, after which the caustic soda is removed by draining 40 in a settling tank or any suitable apparatus. After the draining has been accomplished, the caustic soda retained by the pulp is uniformly washed out with purified water until the pH is between 7.0 and 10.0 units. It is important that 45 any treatment of the cellulose in strong NaOH solutions be carried out uniformly with respect to each fiber so that the effect of the treatment is fully reflected in the condition of the individual fibers rather than in the average condition 50 of the mass of cellulose as a whole. The uniform physical state of the individual fibers imparted by the mercerizing treatment is an especially favorable condition for subsequent reaction; for example, nitration, and it is necessary 55 to carefully maintain this condition throughout the remaining processing steps of the purification treatments.

The pulp may be classified to remove fines 60 which is the term used to include cell wall debris, parenchyma cells, fragments of same, fragments of fibers and vessels, and adsorbed materials from the cellulose fibers, and at the same time to further reduce the ash content. This classification may be practiced at any convenient or economical step in the purification procedure, depending 65 on the type of pulp desired. For example, after mercerization, a pulp is classified through an 80 mesh Allegheny metal screen. An especially efficient apparatus for effecting the desired separation 70 consists of a rubber lined tank equipped with agitation of Allegheny metal construction, and an Allegheny metal 80 mesh screen over the top of the vessel. The pulp, as a 1%-2% slurry in purified water, is fed continuously into the tank, the level being maintained at such a height that

the agitation throws the slurry against the screen covering and imparts thereto a pulsating action. The continuous agitation prevents the formation of a mat of pulp on the screen; the pulsating action imparted to the slurry discharges the fines through the screen, and the water in the slurry washes the fines from the upper surface of the screen, which is installed at a slight angle for this purpose.

The long-fibered fraction of the pulp is discharged into an appropriate vessel from the classification tank and then to further reduce the ash content, is treated with  $\frac{1}{4}$  percent (0.25%) concentration of hydrochloric or acetic acid at a 3% consistency for 15 minutes at 20°-23° C., after which the pulp is washed with purified water which is of a pH of 7.2-7.6, low in total solids, iron, copper and other metallic impurities, until the acid concentration has been reduced to approximately 0.05% and then dewatered.

Sufficient hot purified water at 60°-65° C. and at a pH of 7.0-8.0 is then added to give a 3% slurry and the mass agitated for 30 minutes, de-watered by centrifuging, and then cooled to approximately 20° C. with cold purified water and de-watered again to about 50% moisture content. The water wet pulp will have a pH between 7.0 and 8.0 units.

All of the preceding treatments are preferably carried out under precise conditions of control with respect to:

1. Concentration of the solutions
2. Quality of the reagents, including water
3. Consistency of the pulp slurries
4. pH of treating liquors and wash waters
5. Time and temperature of treatments
6. Cleanliness of air throughout buildings and equipment
7. Minimum exposure of pulp to air, especially under alkaline conditions and/or higher than room temperature
8. Maintenance of pulp moisture above approximately 50%.

The alpha cellulose content of the resulting product is greater than 98% and soda solubility is less than 4%.

The desirable point in the purification treatment for controlling the cuprammonium viscosity of the cellulose is during the calcium hypochlorite treatment preceding the treatment with 7% NaOH at 100° C. It is understood that variations in the wood and in the methods of digestion may result in pulps varying quite widely in their viscosity values immediately subsequent to digestion and prior to the first chlorine water treatment. Nevertheless, the nature of any particular lot of wood is determined and the digestion adjusted to give crude pulps having substantially uniform viscosity values. The chlorination and the subsequent causticization are also carefully controlled so that the viscosity values are not less than those of the raw pulp immediately after the digestion.

The precise control of viscosity is attained by 65 adjusting the conditions in the hypochlorite bleaching treatment. It is understood that reduction of viscosity depends upon:

1. Temperature of the hypochlorite solution
2. Consistency of pulp slurry
3. Time of bleaching
4. Concentration of calcium hypochlorite
5. pH of the solution throughout the bleaching.

Of these, a variation of temperature, time and 75

concentration gives the greatest latitude in obtaining the desired viscosity.

In the foregoing example, the consistency of the pulp in the various treatments may vary quite considerably, depending upon the type of equipment in which the treatments are carried out; the only requisite being that the pulp receive uniform treatment with the reagent employed. In the 1% boiling treatment following chlorination,

10 the time required to bring the temperature of the mass of pulp and alkaline liquor to 100° C. is preferably held between 30 and 120 minutes. In the mercerizing treatment, the time of mercerization is not critical; for instance, it may vary from 15  $\frac{1}{2}$ -4 hours.

#### Example B

In this example is described the purification of unbleached kraft pulp having the following analysis:

|    |                 |                         |      |
|----|-----------------|-------------------------|------|
| 20 | Alpha           | approximate per cent    | 92   |
|    | Soda solubility | do                      | 9    |
|    | Viscosity       | approximate centipoises | 32   |
|    | Ash             | approximate per cent    | *0.8 |
| 25 | Bleachability   | do                      | 36   |
|    | Pentosan        | do                      | 11   |

\* In the specific example being quoted, the ash contained iron and copper in amounts of 48 P. P. M. and 10 P. P. M., respectively, based on the dry weight of cellulose.

30 The pulp, after complete defibering, was chlorinated by adding an amount of chlorine in the form of chlorine water equivalent to 16% of the bleach value of the pulp, and the mass allowed to stand for the total time of 45 minutes. At the

35 end of this period of time, the pulp was washed thoroughly with water and sufficient sodium hydroxide added to the pulp slurry to form a 1% caustic solution. The pulp was then boiled in this caustic solution for  $\frac{1}{2}$  hour. The pulp was then washed neutral with water and treated at 2.7% consistency with 6% calcium hypochlorite based on the weight of oven dry pulp for 4 hours. The pulp was then dewatered, washed with water and treated at 3% consistency at 100° C. for 3 hours in

40 7% sodium hydroxide solution and again washed with water. This 7% boiling treatment resulted in a pulp of considerably lighter color. The pulp was then bleached with 0.5% bleaching powder in the form of calcium hypochlorite for  $\frac{1}{2}$  hour at about 20° C. The pulp was then dewatered, washed and treated at 3% consistency for 1 hour at 20°-25° C. in 13.7% sodium hydroxide solution. The pulp was then again thoroughly washed with water and treated with 13.7% sodium hydroxide solution for 1 hour at 3% consistency at 20°-25° C.

45 All of the washing treatments were carried out on an Allegheny 60 mesh wire screen, thus accomplishing to a certain extent in each washing step a removal of a part of the undesirable "fines." 50 The finished product had an analysis as follows:

|                 |             |      |
|-----------------|-------------|------|
| Alpha           | per cent    | 99.4 |
| Soda solubility | do          | 2.7  |
| Viscosity       | centipoises | 15.1 |
| Ash             | per cent    | 0.23 |
| Iron            | P. P. M.    | 43.9 |
| Copper          | do          | 14.0 |
| Bleachability   | per cent    | 0.25 |
| Pentosan        | do          | 2.5  |

55 70 This product is admirably suited for the preparation of high quality viscose, cellulose nitrate, or even paper where great stability of product is important.

Alpha cellulose is defined as that portion of a sample of cellulosic material not dissolved by

17.5% sodium hydroxide solution at 20° C., determined by a refinement of the method described by H. F. Lewis in "Technical Association Papers," series XVII, #1, 436 (1934), described in copending application of Lyle Sheldon et al., S. N. 81,844, filed May 26, 1936, pages 11-13.

Bleachability of cellulose, as used herein, is a measure of the materials oxidizable by potassium permanganate in the presence of an acid under specific conditions, and is expressed in terms of standard bleaching powder containing 35% available chlorine. A detailed description of the method, including the conversion table for expressing the permanganate number in terms of percent bleaching powder of 35% available chlorine, was published by T. A. F. P. I., series XVII, #1, 146 (1934), "Permanganate Number of Pulp" by R. N. Wiles.

Cuprammonium viscosity, as used herein, means the viscosity number or value obtained according to the following method: The cuprammonium solution was prepared by the action of air on electrolytic copper in the presence of strong ammonia water. The copper concentration of the solutions employed for viscosity determinations was 30,  $\pm 2$  g. per liter, and the ammonia content was 165 g.,  $\pm 2$  g. per liter. The concentration of cellulose employed was 0.6 g. (oven dry basis) per 100 cc. of cuprammonium solution. The cellulose sample for this determination was dried at 70° C. to 4% moisture content. After weighing out 0.6 g. (oven dry basis), the sample was moistened, squeezed to a uniform weight of 2 g. and then dispersed in cuprammonium solution in an atmosphere of hydrogen from which oxygen had been completely removed. The viscosity measurements were made at 25° C. with a modified Ostwald pipet, constructed according to the specifications of the American Chemical Society Committee on the Viscosity of Cellulose (Journal of Industrial & Engineering Chemistry, I, #49; 1929). The time of flow in seconds was converted to centipoises on the basis of the calibration of the pipet with oils of known viscosity in centipoises obtained from the United States Bureau of Standards.

This application is a continuation in part of application Serial Number 39,113, filed September 4, 1935.

Having set forth the process in detail, what I claim is:

1. The process of preparing a homogeneous highly permeable derivative wood pulp having an alpha cellulose content greater than 98 percent and a soda solubility of less than 4 percent which comprises gradually removing the non-cellulosic content from wood by preparing an alkaline digested unbleached pulp having the non-cellulosic content uniformly distributed throughout the fibers by first boiling wood subdivisions in an alkaline delignifying liquor until the air is removed from the woody interstices and then heating said subdivisions submerged in said alkaline liquor to form a completely defiberable pulp, chlorinating said alkaline digested pulp with an amount of chlorine in the form of chlorine water only sufficient to react with the lignin content of the pulp, washing the pulp with water and thereafter gradually increasing the alpha cellulose content and decreasing the soda soluble content of the fiber by subjecting the chlorinated pulp to a succession of chemical refining treatments in an alkaline medium including treatment with an alkaline solution of less than 7 percent concentration, treatment with hypochlorite solution at a pH maintained greater than 7.0 for a time and at a temperature sufficient to control and lower the cellulose viscosity to the desired value, treatment with a caustic soda solution of 5 percent to 9 percent concentration to remove non-cellulosic impurities, bleaching to whiteness with a dilute hypochlorite solution at a pH maintained greater than 7.0, and treatment with a 10 percent to 18 percent solution of caustic soda under mercerizing conditions, each of said chemical refining treatments being followed by a thorough water washing treatment.
2. The process as set forth in claim 1 in which the alkaline reagent in the delignifying liquor and subsequent alkaline treatments is sodium hydroxide.

FREDRICH OLSEN.